

Aug. 19, 1952

H. C. HARSH, ET AL  
PROCESS OF PRODUCING MULTILAYER COLOR NEGATIVES CONTAINING  
MASKING IMAGES FOR COLOR CORRECTION PURPOSES  
Filed March 24, 1950

2,607,681



INVENTORS  
HAROLD C. HARSH  
JOSEPH S. FRIEDMAN  
BY *Henry B. Fellows*  
*Henry B. Fellows*  
ATTORNEYS

## UNITED STATES PATENT OFFICE

2,607,681

## PROCESS OF PRODUCING MULTILAYER COLOR NEGATIVES CONTAINING MASKING IMAGES FOR COLOR CORRECTION PURPOSES

Harold C. Harsh and Joseph S. Friedman, Binghamton, N. Y., assignors to General Aniline & Film Corporation, New York, N. Y., a corporation of Delaware

Application March 24, 1950, Serial No. 151,826  
In Canada May 27, 1947

12 Claims. (Cl. 95—2)

1

This invention relates to color photography, and more particularly to a process of producing multilayer color negatives containing masking images for color correction purposes.

In the production of color prints from multilayer color negatives, the color negative consists of yellow, magenta, and cyan images in the different layers. The cyan image represents the red, the magenta image the green, and the yellow image the blue record of the original subject. Color positive prints or transparencies may be obtained from such color negatives by direct printing onto a multilayer color positive film or paper, or by making color separation negatives which are used for making the color positive prints. These color negatives do not as a rule completely satisfy the spectral requirements for trichromatic color reproduction. For instance, the magenta colored image, formed by the imposition of green light upon the green sensitive layer, records the green densities. This image should transmit the blue and the red primaries, completely. To the extent to which it absorbs blue light, it superimposes a pattern of the green densities upon the blue, with consequent color falsification. This color falsification makes itself manifest when the color negative is to be printed. That part of the exposure which is due to blue light, and which should form a record only of the image in the yellow layer in the negative, forms a record of the yellow image admixed with the record of the magenta. The image in the blue sensitive part of the copy material is, therefore, very impure, and serious color degradation results.

It is possible to overcome this defect if procedures are devised to register a pattern of the magenta dye image, equal in intensity to the degree to which the magenta dye absorbs blue light, but opposite in character, with the yellow dye images. In a similar manner the cyan dye image can be corrected for its blue absorption. These masks or modifying images can be yellow in color, as suggested by the prior art, or they can be a neutral gray, composed of dye or silver.

Numerous methods have been proposed for making corrections in these dye images. Generally, these methods are characterized by the fact that the mask is on a separate piece of film, and must be registered with the original by manual or mechanical means. This creates problems of registry arising from the dimensional variations of film as it ages, and problems of definition arising from lack of optical contact between original and mask, Newton rings, etc. It is desirable,

2 therefore, to have the mask integral with the original. To accomplish this, it has been proposed to place an auxiliary emulsion layer within the pack in which the mask could be formed. 5 While this gives a desirable result, it introduces complications into the structure and the preparation of the monopack material. Since the masking image is opposite in character to the one that it is desired to modify, emulsions with special properties have to be used.

To eliminate this complication, it was proposed in British Patent 541,266 to utilize the residual silver halides in the emulsion after the latent image has been processed to a dye image, and to convert the residual halides, after a proper exposure, into a black and white silver mask. The procedure disclosed to accomplish the formation of a mask was to treat the film after negative color development in a bleach bath to convert the silver to silver chloride, to remove the silver chloride by treatment with ammonia or ammonium sulfite, then to expose the untouched residual silver bromide to white light, and develop in an M. Q. developer that yields a silver image. When processed in this manner, there are formed silver images in each of the layers of the color film. This may be desirable under certain conditions, but for certain purposes the presence of a mask representing an image of the yellow dye pattern is harmful and undesirable. This was recognized by the British patentee and he specifically states in his specifications that the bleach, to be used to effect a conversion of the silver to silver chloride, be of such a mild nature that it does not destroy the color sensitivities of the green and red sensitive layers. After treatment with such a mild bleach solution, it becomes possible to selectively expose the red and/or green sensitive layers, so that masking images be formed only in these parts.

45 The restriction that a bleach be used that is so mild that it does not destroy the color sensitivity of the green and red layers, severely limits the operator using the material and the manufacturer who makes it. The patentee cites a number of sensitizing agents that could be used, which will not be destroyed by the extremely mild agents he mentions. But, generally, subjecting an optically sensitized film to the action of an oxidizing agent reduces the color sensitivity of that material almost to the vanishing point. To effect a selective exposure in the green and red sensitive layers would require such long durations as to make the procedure impractical unless

special sensitizers be used which are not so affected.

It is, therefore, an object of the present invention to provide a method for obtaining dye images in multilayer photographic color negative materials that contain, at the same time, masking images composed of silver salts which correct for the color deficiencies of the dye images.

A further object is to provide a method for obtaining color corrected color negative materials wherein the color correction is integrally bound with the dye images.

Other objects and advantages of this invention will be apparent by reference to the foregoing specification, in which its preferred details and embodiments are described.

The foregoing objects are accomplished by fixing an exposed and developed photographic color negative film for a period of time ranging from  $\frac{1}{2}$  to  $2\frac{1}{2}$  minutes, in a bath consisting of the following composition:

|                                | Grams |
|--------------------------------|-------|
| Ammonium or sodium thiosulfate | 100   |
| Sodium sulfate                 | 100   |
| Water to make 1 liter.         |       |

All of the silver halides remaining in the uppermost (blue sensitive) layer are removed, leaving intact the silver halides in the other two layers. The sodium sulfate reduces the penetration of the thiosulfate and limits its action to the uppermost layer. The fixed film is then washed with water.

It is now possible to effect a non-color selective masking image in the cyan and magenta layers by bathing the film in an aqueous solution of potassium or sodium iodide. This solution converts the residual silver halides in the green and red sensitive layers into silver iodide, which will act as a mask. To achieve a more opaque image, the iodide bath may be replaced by a sulfide bath of the type used to form silver sulfide images, such as a 1% solution of sodium sulfide. After conversion to iodide or sulfide, the film is treated with a solution or solutions that will convert the silver present in the negative, filter, or anti-halation layer, to a form which is soluble in hypo, so that salts like silver ferrocyanide, silver chloride or bromide can be readily removed before any action on the iodide or sulfide becomes evident. A bleach bath such as:

|                        | Grams |
|------------------------|-------|
| Potassium ferricyanide | 40    |
| Sodium bromide         | 100   |
| Water to make 1 liter. |       |

will convert the silver to silver bromide without affecting either silver iodide or silver sulfide to any appreciable extent.

The procedure as outlined above comprises the following steps:

1. Exposure of the color negative film.
2. Development of the latent images with a color developer.
3. Continued development of the film with a sulfite-containing black and white developer to achieve gamma infinity in all three layers. Although the continued black and white development may be optional, its inclusion, however, is desirable since it controls the quality of the final masking image.
4. Fixation by controlled diffusion of the residual halides in the top or blue sensitive layer of the film.
5. Conversion of the residual silver halides in

the green and red sensitive layers to silver iodide or silver sulfide.

6. Conversion of the negative and any other colloidal silver to a silver halide or ferrocyanide.

7. Fixation of all reformed silver salts in the film.

8. Washing and drying.

The foregoing description of our invention will be more apparent from the following examples which are set forth merely to illustrate the invention and should not be construed as a limitation thereof.

*Example I*

A multilayer photographic color film such as prepared according to United States Patents 2,179,228; 2,179,239; 2,186,849; 2,220,187, and 2,357,388, was exposed to a colored object and then developed for 15 minutes in a color developer of the following composition:

|                                        | Grams |
|----------------------------------------|-------|
| Diethylamino aniline                   | 1.5   |
| 2-amino-5-diethylaminotoluene mono HCl | 1.0   |
| Sodium sulfite                         | 0.5   |
| Sodium carbonate                       | 67.5  |
| Potassium bromide                      | 2.5   |
| Hydroxylamine HCl                      | 0.5   |
| Water to make 1 liter.                 |       |

This development resulted in the formation of negative silver and color images at the exposed portions of the multilayer film. The color developed film was then shortstopped in a 1% solution of acetic acid containing 1% sodium acetate, washed for 10 minutes, and then fixed for 1 $\frac{1}{2}$  minutes in a solution of the following composition:

|                             | Grams |
|-----------------------------|-------|
| Sodium thiosulfate          | 100   |
| Sodium sulfate (dehydrated) | 100   |
| Water to make 1 liter.      |       |

By this fixing treatment the residual silver halides in the uppermost blue sensitive layer were removed. The silver halides in the remaining layers were not materially affected. In this fixing bath the function of the sulfate is to prevent the rapid diffusion of the fixing bath into the depth of the film. Any other agent, such as alcohol, glycerin, sugar, etc., which function in like manner, can be used.

The film was washed in running water for 10 minutes to remove excessive fixing bath, and then subjected to the action of a 1% solution of potassium iodide, for a period of 10 minutes. In this treatment, the positive silver halide images present in the cyan and magenta layers were converted into silver iodide, which is stable and non-sensitive to the action of light.

All the metallic silver present in the various layers was then converted into a silver salt, such as silver ferrocyanide, by the action of a 10% solution of potassium ferricyanide. Instead of employing aqueous solutions of potassium ferricyanide, as the oxidizing agents, other solutions of the commonly known oxidizing agents which convert the silver to a silver salt other than silver iodide, may be used, such as, for example, ferric chloride, copper sulfate in the presence of bromide or chloride ions, and the like. The bleached film was washed in running water for several minutes and treated with a normal fixing bath for 5 minutes, washed, and then dried.

In the normal fixing bath, the rate of fixation of the silver salts, such as silver chloride, silver bromide, silver ferrocyanide, and the like, is so

much greater than the dissolution of silver iodide that to all intents and purposes, the action can be considered as affecting only the silver chloride, silver bromide and silver ferricyanide, thus leaving the silver iodide image substantially unimpaired. By this means, the silver iodide positive images in the cyan and magenta layers, serve as masking images to provide for color correction in printing with a minimum of processing steps and a considerable saving of time in comparison with other masking methods.

*Example II*

Example I was repeated with the exception that after color development, the film was further developed in a non-staining black and white developer such as:

|                        | Grams |
|------------------------|-------|
| Pyrogallic acid        | 5     |
| Sodium sulfite         | 30    |
| Sodium carbonate       | 10    |
| Potassium bromide      | 2     |
| Water to make 1 liter. |       |

or any other known non-staining black and white developer. This development was carried on to gamma infinity (the highest obtainable contrast of a film) so that all exposed silver halide grains were developed.

The colored and black and white developed film was then differentially fixed and processed through to completion in the manner set forth in Example I. This procedure has the advantage over the procedure in Example I in that it removes all danger of having a residual negative silver image developed in the final or masking development, since all silver halide unexposed in the first exposure, is exposed and converted to metallic silver thereby.

*Example III*

Example I was repeated with the exception that a 0.5% solution of sodium sulfide was used in place of potassium iodide. The masking image obtained showed a greater opacity.

*Example IV*

Example II was repeated with the exception that a 1.5% solution of sodium sulfide was used in place of potassium iodide.

In the accompanying drawing, the figure is a flow diagram representing enlarged sectional views of a film showing the method of forming a masked image according to our invention. Views A, B, C, and D of the figure illustrate the changes taking place in the film during the various steps of processing.

As shown in the figure, 10 is a transparent base or support having superposed thereon, layers 11, 12, and 14 containing cyan, magenta and yellow color images, respectively. Layer 13 represents a filter layer.

A illustrates a section of the multilayer color film which has been exposed and color developed.

B illustrates the same multilayer color film after the residual silver halide in the top layer has been removed by selective fixation.

C illustrates the same multilayer color film after the conversion of the residual silver halides in the two lower layers to silver iodide or silver sulfide.

D illustrates the same multilayer color film after bleaching and fixation.

It will be noted that masking images consisting of silver iodide or silver sulfide are only formed in the magenta and cyan layers.

Obviously, the practice of the present invention is not to be limited to the processing of multilayer photographic color film of the type set forth in the examples. Multilayer photographic film such as prepared according to United States Patents 2,269,158; 2,266,443; 2,272,191; 2,284,877; 2,289,803; 2,304,940; 2,311,020; 2,350,380; 2,397,864-5-6 and 7, and the like, can also be processed into color negatives containing masking images in accordance with the present invention. Various other modifications will occur to those skilled in the art which, however, do not depart from the spirit and nature of this invention, and we do not intend to be limited in the patent granted except as required by the prior art and in the following claims.

This application is a continuation-in-part of our application Serial No. 703,480, filed on October 16, 1946.

We claim:

1. In the production of subtractively colored negatives with correction printing masks, integrally bound therein, for multilayer film having silver halide emulsions containing color formers and being respectively sensitized to the blue, green, and red regions of the spectrum, by exposing said multilayer film to a colored object and color developing the same, the improvement which comprises selectively fixing the residual silver halides in the blue sensitive layer, converting the residual light sensitive silver halides in the other emulsion layers into light insensitive silver salts selected from the group consisting of silver iodide and silver sulfide, and removing all metallic silver.
2. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises selectively fixing the residual silver halides in the blue sensitive layer, converting the residual light sensitive silver halides in the other emulsion layers into light insensitive silver salts selected from the group consisting of silver iodide and silver sulfide, and removing all metallic silver.
3. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises selectively fixing the residual silver halides in the blue sensitive layer, converting the residual light sensitive silver halides in the other emulsion layers into light insensitive silver salts selected from the group consisting of silver iodide and silver sulfide, and removing all metallic silver.
4. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises selectively fixing the residual silver halides in the blue sensitive layer, converting the residual light sensitive silver halides in the other emulsion layers into light insensitive silver salts selected from the group consisting of silver iodide and silver sulfide, and removing all metallic silver.

of coupling with the color former in the layer, for a time sufficient to bring the development to gamma infinity, selectively fixing the residual silver halides in the blue sensitive layer, converting the residual silver halides in the magenta and cyan layers to insoluble silver salts selected from the group consisting of silver iodide and silver sulfide, converting all metallic silver to a silver salt soluble in hypo, and treating the film with hypo to remove the silver salt thus formed.

5. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises developing the said color developed film in a non-staining developer incapable of coupling with the color former in the layer, for a time sufficient to bring the development to gamma infinity, selectively fixing the residual silver halides in the blue sensitive layer, converting the residual silver halides in the magenta and cyan layers, to silver iodide, converting all metallic silver to a silver salt soluble in hypo, and treating the film with hypo to remove the silver salt thus formed.

6. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises developing the said color developed film in a non-staining developer incapable of coupling with said color formers, for a time sufficient to bring the development to gamma infinity, selectively fixing the residual silver halides in the blue sensitive layer, converting the residual silver halides to silver sulfide, converting the metallic silver in all layers to a hypo soluble silver salt, and treating the film with hypo to remove the silver salt thus formed.

7. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises developing the said color developed film in a non-staining developer incapable of coupling with said color formers, for a time sufficient to bring the development to gamma infinity, selectively fixing the residual silver halides in the blue sensitive layer with an aqueous solution containing hypo and a member selected from the class consisting of alkali sulfates, water miscible alcohols, sugar, and glycerin, and converting the residual light sensitive silver halides in the other emulsion layers into a light insensitive form by treating with a member selected from the class consisting of aqueous solutions of alkali sulfides and alkali iodides.

8. In the production of subtractively colored negatives with correction printing masks, integrally bound therein, for multilayer film having silver halide emulsions containing color formers and being respectively sensitized to the blue, green, and red regions of the spectrum, by ex-

posing the said multilayer film to a colored object and color developing the same, the improvement which comprises developing the said color developed film in a non-staining developer incapable of coupling with said color formers, for a time sufficient to bring the development to gamma infinity, selectively fixing the residual silver halides in the blue sensitive layer, with an aqueous solution containing hypo and sodium sulfate and converting the residual light sensitive silver halides in the other emulsion layers into a light insensitive form by treatment with an aqueous solution of potassium iodide.

9. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises selectively fixing the residual silver halides in the blue sensitive layer, converting the residual silver halides in the other emulsion layers to an insoluble silver salt selected from the class consisting of silver iodide and silver sulfide, and removing all developed silver by bleaching and fixing to produce positive silver images in the magenta and cyan layers.

10. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises selectively fixing the residual silver halides in the blue sensitive layer, converting the residual silver halides in the magenta and cyan layers to silver iodide by treatment with an aqueous solution of potassium iodide, converting all metallic silver into silver ferrocyanide with an aqueous solution of potassium ferricyanide, and treating the film with hypo to remove the silver ferrocyanide thus formed.

11. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises selectively fixing the residual silver halides in the blue sensitive layer with an aqueous solution containing hypo and sodium sulfate, converting the residual silver halides to silver sulfide by treatment with an aqueous solution of sodium sulfide, oxidizing all metallic silver with an aqueous solution of potassium ferricyanide, and treating the film with hypo to remove the silver ferrocyanide thus formed.

12. In the production of subtractively colored negatives with correction printing masks, integrally bound therein, for multilayer film having silver halide emulsions containing color formers and being respectively sensitized to the blue, green, and red regions of the spectrum, by exposing the said multilayer film to a colored object and color developing the same, the improvement which comprises developing the said color developed film in a non-staining, sulfite-containing developer incapable of coupling with the color former in the layer, for a time sufficient to bring

the development to gamma infinity, selectively fixing the residual silver halides in the blue sensitive layer, with an aqueous solution containing hypo and sodium sulfate, converting the residual silver halides to silver sulfide by treatment with an aqueous solution of sodium sulfide, oxidizing all metallic silver with an aqueous solution of potassium ferricyanide, and treating the film with hypo to remove the silver ferrocyanide thus formed.

## REFERENCES CITED

The following references are of record in the file of this patent:

## UNITED STATES PATENTS

| Number    | Name         | Date          |
|-----------|--------------|---------------|
| 2,203,653 | Evans        | June 4, 1940  |
| 2,431,996 | Duerr et al. | Dec. 2, 1947  |
| 2,476,541 | Friedman     | July 19, 1949 |

10

## FOREIGN PATENTS

| Number  | Country       | Date          |
|---------|---------------|---------------|
| 517,020 | Great Britain | Jan. 18, 1940 |
| 541,266 | Great Britain | Nov. 20, 1941 |

HAROLD C. HARSH.  
JOSEPH S. FRIEDMAN.